

## UNITED STATES PATENT OFFICE.

EDWARD R. ALLEN AND WILFORD E. KAUFMANN, OF EAST ORANGE, NEW JERSEY,  
ASSIGNORS TO E. I. DU PONT DE NEMOURS & COMPANY, OF WILMINGTON, DELA-  
WARE, A CORPORATION OF DELAWARE.

## DISPERSING POWDER AND PROCESS OF MAKING.

No Drawing.

Application filed July 3, 1925. Serial No. 41,432.

This invention relates to the production of quickly wetting and dispersing powders of the ordinary pigments, which powders are adapted to be used in the art of glazing and coating paper and in the wall paper industries, as well as in the preparation of so-called "water colors" in general. These powders as prepared by us possess the novel and surprising property of mixing readily in water. By reason of this property, the new powders give satisfactory results in many types of industrial operations, in which the use of powders prior to our invention has been impractical or impossible, since, when the ordinary dried powders were used they would not disperse appreciably or even wet up readily in water, and would consequently produce streaked and uneven effects on the goods. Full or satisfactory tintorial value was by no means obtained from the pigment in such powders, and it was necessary to employ instead "pulps," that is, pigments in the form of pastes or wet cakes.

The use of pulps also, however, entails several disadvantages, among them being the danger of their freezing in cold weather, the necessity of transporting them in waterproof containers, and their bulk and excessive weight due to their water content which renders them inconvenient to handle and expensive to ship. With this state of the art in mind we have succeeded in producing dry powders which have none of the objectionable features of a paste, and have also developed a method for their manufacture. These powders when mixed thoroughly with water, disperse in an entirely satisfactory manner.

This result we accomplish by the very thorough incorporation into the original pulp of suitable colloidal substances, either water-absorbing or true dispersing agents, which substances impart to the pigment the property of wetting up in water after drying. This effect is produced to a certain extent with such substances as starches, gums, and dextrines, but more effectively by the use of true dispersing agents such as soaps, Turkey red oil, licorice, saponin, and "soap bark extract" of commerce, consisting largely of saponin.

In the manufacture of our powders any of the ordinary water insoluble pigments generally employed in the preparation of water colors as lead chromate, lead sulphate, lead phosphate, Prussian blue, etc., may be employed. In general, the pigment in the form of the original pulp or wet cake is mixed with the same amount or more of water to form a paste, and is worked up with the dispersing agent by stirring or vigorous agitation until the latter is thoroughly incorporated therewith. With continued agitation the paste is converted into a smooth foamy mass of increased volume, the amount of increase depending upon the particular dispersing agent and the amount thereof employed. In general, the dispersing agent is added in such quantities as to approximate from 1% to 10% of the weight of the dry pigment. The smooth foamy mass resulting from the use of saponin, licorice, soap bark extracts and soap may approximate from two to three times the volume of the original charge. This mass is now dried. Such drying may be affected in any ordinary manner without regard to a particular apparatus; as by a current of warm air, on the surface of a heated drum, in a belt drier or by any other appropriate method. The dried mass is now ground to a powder which is the final product.

The following specific examples will serve to illustrate our process as applied to several representative pigments, it being understood that we do not confine ourselves to the proportions or materials hereinafter mentioned:

*Example 1. Production of a dispersing powder of a chrome yellow.*

A smooth paste (consisting of 50-85% water) of the ordinary pigment known in the trade as lemon yellow, and consisting of a mixture of lead chromate, lead sulphate and lead phosphate, is stirred up in the presence of saponin equal to 1 to 10% of the weight of dry pigment present. In a short time a smooth foam results which is 2 to 3 times the volume of the original charge. This foam when dried grinds to a powder which shows considerable dispersion when thrown directly into water, and when stirred up for some hours with an equal weight of water, gives a smooth foaming pulp which

disperses equally as well in a large volume of water as does the original undried pulp.

*Example 2. Production of a dispersing powder of a chrome yellow.*

The procedure is exactly the same as in Example 1, except that a solution of licorice is used in place of the saponin. Slightly less foaming results in connection with this dispersing agent, yet the results from a practical standpoint are essentially the same.

*Example 3. Production of a dispersing powder of a chrome green.*

A smooth paste (30 to 50% solids) is made of a chrome green pigment consisting of 29.73% of lead chromate and 3.26% Prussian blue. To this is added a 50% solution of Turkey red oil (ammonium salt of sulphonated castor oil) in an amount equal to 10% of the weight of the dry content of the paste and the mixture agitated for some hours. The alkalinity of the charge is then carefully neutralized with a watery extract of casein (obtained by boiling up commercial casein with water), stirred an hour or more longer then dried and ground. This product when stirred up with water for some hours or preferably mechanically agitated over night, forms a smooth pulp which disperses in water in a manner comparable to the original pulp.

*Example 4. Product of a dispersing powder of a chrome green.*

A smooth paste (20 to 50% solids) of a chrome green, medium shade, consisting of 29.73% lead chromate, and 3.26% Prussian blue is stirred up in the presence of soap bark extract containing solids equal to 1 to 10% of the solids of the pigment paste. With vigorous agitation the paste approximately triples in volume as was true in the case cited under Example 1. The foamy product when dried and ground disperses appreciably when introduced into water, but to an extent equal to the original pulp if stirred up with water under the conditions described in Example 1.

*Example 5. Production of a dispersing powder of Prussian blue.*

A paste of Prussian blue (approximately 60% water) is stirred up with good agitation and partially dispersed with sodium or potassium oxalate, (the dispersing action of oxalates on Prussian blue is well known, Bancroft, Applied Colloid Chemistry p. 177), equal in weight to 2% of the solid content of the pigment paste. Soap bark extract containing solids equal to 1 to 10% the total solids content of the pigment is then added and the whole stirred thoroughly until a good foam structure is produced. During this agitation it is necessary to add

water gradually so that the final foam is about 85% water. This product when dried and ground will give when stirred up with water under the conditions described under Example 1 a smooth pulp which will disperse in water equally as well as the original undried pulp.

It will be understood that by the term "dispersing agent" as used in the appended claims and throughout the specification we intend to indicate those substances as starches, gums and dextrines which may be considered to act at least in part by virtue of their water retaining properties, thus preventing the particles of pigment from adhering or forming into aggregates during drying and which, by their swelling properties, tend to break up any aggregates found when placed in water, as well as to indicate the so-called "true dispersing agents" which may be used in smaller amounts and are generally considered to act largely by virtue of their influence on surface tension whereby they are thought to distribute themselves in infinitesimal films over the surfaces of the particles.

We claim:

1. The process of preparing a dry water dispersible powder from an inorganic pigment not readily miscible with water which comprises agitating an aqueous mixture containing said pigment and an amount of a dispersing agent between 1% and 10%, by weight of the pigment, to produce a homogeneous mass, drying said mass and grinding it to a colloid like condition.

2. A process for preparing a dry water dispersible powder from a water insoluble pigment, which comprises agitating said pigment with water and a dispersing agent until the agent is thoroughly incorporated, slowly adding water during such agitation to produce a mass of foam comprising about 85% water, drying the resulting mass and grinding the dried mass to a powder.

3. A process for preparing a dry water dispersible powder from a water insoluble inorganic pigment which comprises mixing a dispersing agent with an aqueous paste of said pigment, said agent being added in such quantity as not to exceed 10% by weight of the dry pigment, agitating to produce a homogeneous mass of foam, drying said mass and reducing the dried mass to a powder.

4. In a process for preparing a dry water dispersible powder from an aqueous paste of a water insoluble inorganic pigment the steps of adding saponin to said paste and then converting the paste to a mass of foam.

5. In a process for preparing a dry water dispersible powder from an aqueous paste of a water insoluble inorganic pigment the steps of converting said paste to a mass of foam and drying said mass.

6. In a process for preparing a dry water dispersible powder from an aqueous paste of a water insoluble inorganic pigment the steps of converting said paste to a mass of 5 foam, drying said mass and grinding the dried mass.
7. A process for preparing a dry water dispersible powder from a water insoluble inorganic pigment which comprises adding 10 a foam producing dispersing agent to an aqueous paste of said pigment, agitating until a mass of foam is formed, drying, and grinding the dried mass.
8. In a process for preparing a dry water dispersible powder from an aqueous paste of a water insoluble inorganic pigment the steps of incorporating with said paste a foam producing dispersing agent and then agitating the mixture into a mass of foam.
9. A process for preparing a dry water dispersible powder from an aqueous paste of a water insoluble inorganic pigment which comprises adding a foam producing dispersing agent to said paste, agitating to produce 20 a mass of foam and converting said mass to a powder.
10. A process for producing a water insoluble inorganic pigment in dry, water dispersible form which comprises agitating an aqueous paste of said pigment and a foam producing dispersing agent until a mass of foam results, and reducing said mass to a dry colloid-like powder.
11. A dry colloid like powder obtained 30 by agitating an aqueous mixture of an inorganic pigment not readily miscible with water and an amount of a dispersing agent between 1% and 10%, by weight of the pigment, to produce a homogeneous mass, drying said mass and grinding, said powder being characterized by the property of dispers- 35
- ing readily in water to form a smooth pulp.
12. A dry colloid like powder obtained by agitating an aqueous mixture of an inorganic pigment not readily miscible with 45 water and an amount of a foam producing dispersing agent between 1% and 10%, by weight of said pigment until a homogeneous mass approximating from two to three times the volume of the original mixture 50 results, drying said mass and grinding, said powder being characterized by the property of dispersing readily in water to form a smooth pulp.
13. A water dispersible powder comprising a uniform mixture of a water insoluble inorganic pigment and a foam producing dispersing agent, said agent being present in an amount less than 10%, by weight, of the 55 pigment.
14. A water dispersible powder comprising a uniform mixture of a water insoluble inorganic pigment and saponin, said saponin being present in an amount less than 10%, by weight, of the pigment.
15. A dry colloid like powder obtained by agitating an aqueous mixture of an inorganic pigment not readily miscible with water and a foam producing dispersing agent until a mass of foam is produced, drying said mass and grinding, said powder being characterized by the property of dispersing readily in water to form a smooth pulp.
16. A water dispersible powder comprising an inorganic pigment, the particles of said powder having the structure of ground dried foam.

In testimony whereof we affix our signatures.

EDWARD R. ALLEN.  
WILFORD E. KAUFMANN.